

Patented July 12, 1927.

1,635,637

# UNITED STATES PATENT OFFICE.

GEORGE A. RICHTER, OF BERLIN, NEW HAMPSHIRE, ASSIGNOR TO BROWN COMPANY, OF BERLIN, NEW HAMPSHIRE, A CORPORATION OF MAINE.

## PROCESS OF PRODUCING WHITE PULP OF HIGH STRENGTH.

No Drawing.

Application filed July 11, 1925. Serial No. 42,977.

This invention has relation to a novel pulp suitable for the manufacture of high grade bond and ledger papers, comparable in whiteness to ordinary bleached sulphite 5 pulp and in strength to kraft or "sulphate" pulp, and to a process for the production of such pulp in an economical and expedient manner.

For the purpose of giving a clearer and 10 more sufficient understanding of the present invention and the results achieved thereby, it is necessary to consider, in some detail, the subject matter of my application for U. S. Letters Patent Serial No. 749,564, filed 15 November 12, 1924. In that application, the salient feature of discovery, generally stated, is that if wood chips (spruce, for example), are cooked in an acid sulphite solution in which the free  $\text{SO}_2$  and the combined  $\text{SO}_2$  are in substantially equal proportions (or the free  $\text{SO}_2$  less in proportion than the combined  $\text{SO}_2$ ) but are present in sufficient quantity in solution to act upon the encrusting or cementitious content of 20 the wood for a sufficient period of time in a closed digester at a temperature higher than that ordinarily employed in sulphite digestion, a pulp is produced which has marked characteristics and possesses certain features 25 of advantage over the usual or commercial form of sulphite pulp. Such pulp is especially characterized by its light color, extraordinary strength, length of fiber, and its high lignin and pentosan content, and, for convenience of designation, will be termed 30 "strong sulphite pulp," in contradistinction to the ordinary sulphite pulp. Its strength is probably due to its high ligneous and pentosan content, which approximates that 35 of kraft or "sulphate" pulp. The pentosans, probably due to their adhesive or sticky qualities, act as a binder to bind the constituent fibers strongly together, thereby 40 imparting strength to the pulp. However, owing to such high lignin content, the 45 strong pulp is very difficult to bleach, requiring about 25% to 35% of 35% bleach (based on the bone-dry weight of pulp), to produce a bleached product which has the color of ordinary bleached sulphite pulp, but, owing to the use of excess bleach, the strength of the original pulp is materially reduced, probably due to the degradation of a portion of the cellulose into oxycellulose, so that ordinarily it would not be economical

to bleach strong sulphite pulp for the production of a white pulp in competition with ordinary bleached sulphite pulp.

The primary object of the present invention is to produce a white pulp of high 60 strength from "strong sulphite pulp." To attain this object, the present invention must provide for the removal of the ligneous or coloring substance in the pulp without materially affecting its fiber strength or pentosan 65 content. I have discovered that if strong sulphite pulp is treated with an oxidizing solution containing oxidizing agent in such quantity that a removal of lignin is effected without causing a substantial change in the 70 strength of the pulp or its pentosan content, and is subsequently digested at an elevated temperature in an alkaline solution containing alkaline agent in such quantity as to effect a further removal of impurities in the 75 pulp without affecting its strength, a product results which may be whitened with the usual moderate amount of bleach to give a product of extraordinary strength, comparable to that of kraft, and of a whiteness 80 comparable to that of bleached sulphite pulp. I have discovered, moreover, that the alkaline treatment also imparts a softness to the pulp, and accordingly results in a product which shows a considerably higher tear 85 test than the initial "strong sulphite pulp."

In the practice of the present invention, wood chips (spruce, for example) are cooked in a digester, in an acid sulphite solution, preferably sodium bisulphite (or an equivalent bisulphite solution of zinc, magnesium, potassium, or other suitable metal) having a relatively high combined  $\text{SO}_2$  content, say 3% to 4%, with free  $\text{SO}_2$ , no greater in proportion than the combined 90  $\text{SO}_2$ , at a temperature of about 320° F., and a pressure of about 75 to 95 pounds. In certain cases, however, it may be desirable to commence the digestion of the chips in an acid liquor containing, say, about 7% free 95  $\text{SO}_2$  and 4% combined  $\text{SO}_2$ , and relieve the digester of the excess free  $\text{SO}_2$  during the early stages of the cook. Such procedure, while substantially equivalent to that outlined, gives better penetration of the  $\text{SO}_2$  into the chips and tends to promote a more rapid and efficient liberation of fiber. Due to such higher combined  $\text{SO}_2$  content than is ordinarily present in cooking a sulphite stock, the hydrogen ion concentration or ac-

tivity of free  $\text{SO}_2$  is suppressed sufficiently to avoid the usual rather drastic hydrolysis which occurs in cooking sulphite stock, and hence the average length of fiber is greater than when the acid cooking is carried on with a liquor having a normal or usual combined  $\text{SO}_2$  content; whereas, on the other hand, the pulp contains much of the fiber that in an alkaline digestion is dissolved in the alkaline liquor; that is, the strong sulphite pulp contains a greater proportion of the wood than is contained in either sulphate or commercial sulphite pulp. For example, in ordinary commercial operation with the usual acid bisulphite digestion, the yield of pulp is from 43% to 47% of the weight of the dry wood, and in ordinary sulphate or soda digestion, the yield is from 40% to 47% of the weight of dry wood; whereas, according to my process, the yield is from 50% to 55%. Hence, in addition to cellulose fibers, the strong pulp, as indicated, contains a large proportion of lignin and pentosan, the latter by its presence doubtless imparting thereto its high strength characteristic, and the former its property of difficult bleachability.

After the completion of the "4-4" digestion (that is, a digestion in which the acid liquor contains approximately 4% combined and 4% free  $\text{SO}_2$ ) the digester contents are "blown" into a suitable blowpit. The pulp is separated from the spent liquor, and is washed and, if desired, screened as ordinarily, to remove specks, shives, and other like foreign material. The hot spent liquor may be treated, as described in the copending application, for the recovery of heat and chemicals. The washed and preferably screened pulp is then treated at a stock density of about 10%, at approximately room temperature, with an oxidizing of lignin-removing chlorine-containing solution such as one having about 2% to 4% free chlorine, or 3.5% to 7% of 35% bleach ( $\text{CaOCl}_2$ ) based on the bone-dry weight of fiber, for about ten to thirty minutes. The mild treatment with the oxidizing solution promotes a reaction between the ligninous and coloring substance contained in the pulp with the chlorine, forming soluble reaction products, or products which are removed by the subsequent alkaline treatment, and is a selective reaction, the cellulosic and pentosan content, and also the strength of the pulp, remaining substantially unaffected. After the chlorine treatment, the pulp is washed substantially free of chlorine and entrained products of reaction, and may be then treated for further removal of ligninous and coloring substance by the alkaline digestion.

The washed and treated stock is thickened to the desired consistency, as on a wet machine, and is mixed with an alkaline solu-

tion, preferably of a soluble alkali or alkaline earth metal hydroxide, such as caustic soda, containing about 6% to 8% caustic soda, based on the bone-dry weight of fiber, to a consistency desired for carrying out the alkaline digestion, say about 10%. The stock is digested in open tanks under atmospheric pressure, at about 180° to 212° F., for about two to seven hours (depending on the characteristics of the particular stock undergoing treatment and the temperature and concentration of sodium hydroxide employed in digestion) as by blowing live steam thereinto, preferably while being agitated so as to promote a uniform reaction and give a uniform product. While I have found it more economical and expedient to carry out the alkaline digestion in open tanks, it may be stated that equally effective results may be accomplished by digesting the pulp at an elevated temperature in closed digesters, under pressure. The alkaline digestion is also a more or less selective reaction, the less resistance celluloses, the ligninous, resinous, and other coloring matters surviving the chlorine treatment being dissolved by the caustic soda solution and removed from the pulp without materially affecting its strength or pentosan content. The alkaline digestion, moreover, imparts a softness to the pulp, doubtless due to the removal of bleach-consuming constituents and less resistant celluloses therefrom, and the pulp accordingly shows a materially increased tear test. After the alkaline digestion, the stock is washed substantially free from spent liquor and the reaction products. The spent liquor (which may vary in color from weak tea, in the case of low resinous wood, to a dark brown color, in the case of more highly resinous woods) may be treated for the recovery of chemicals.

The washed pulp is then bleached without injury to its fiber strength, by subjecting it from five to ten hours, at a stock density of about 10%, preferably at room temperature, to a hypochlorite bleach solution containing 12% to 15% of 35% bleach ( $\text{CaOCl}_2$ ), based on the bone-dry weight of fiber. The bleached pulp is then washed substantially free from bleaching solution and reaction products, and may be treated with a solution of anti-chlor, as for example, sodium bisulphite, to react with and neutralize the last traces of bleach. The neutral pulp may then be washed free of reaction products. In certain cases it may be desirable to increase the whiteness of the pulp to a maximum. This may be accomplished by treating the bleached and preferably washed pulp without injury to its fiber strength, at approximately room temperature, at a stock density of 6% to 8%, for about two to six hours, with a chlorine solution containing about 0.3% chlorine,

based on the bone-dry weight of fiber. Such superbleaching treatment increases the color to about 100 to 104.

I present herewith a comparative table 5 showing certain characteristics of "4-4" pulp before and after treatment in accordance with the present invention, together with the same characteristics of "sulphate" or kraft pulp, and sulphite pulp:

|                                 | Un-bleached "4-4" pulp | "4-4" pulp after alkaline and bleaching treatment | Usual kraft or "sulphate" pulp | Usual sulphite pulp |
|---------------------------------|------------------------|---------------------------------------------------|--------------------------------|---------------------|
| Mullen strength (beaten)        | 155-190                | 162-170                                           | 155-160                        | 115                 |
| Slowness in min. (beaten)       | 3-8'                   | 10.3-12'                                          | 5-9                            | 10'-15'             |
| Alpha cellulose (%)             | 80.0+                  | 90.1+                                             | -----                          | 85-97               |
| Fiber length (mm.)              | 90-.95                 | .90-.95                                           | 7-.9                           | 6-.7                |
| Tear                            | 140-160                | 240-250                                           | 220-245                        | 140-160             |
| Color                           | Light                  | 100                                               | Brown                          | Light               |
| Pentosan (%)                    | 5.0-7.5                | 5-6                                               | 7-10                           | 3.0-4.5             |
| Yield % (based on initial wood) | 50-55                  | 46%                                               | 42-45%                         | 45-47%              |

From the foregoing table, which represents the average of a number of tests, it will be seen that the strength and tear of the alkaline digested and bleached "4-4" pulp approximates that of kraft or "sulphate" pulp, and has a color similar to that of bleached sulphite pulp. The pentosan content of my pulp, while slightly lower than kraft, together with a long fiber, doubtless imparts thereto its extraordinary strength. It is to be noted that the yield is equal to that obtained by the usual sulphite process, and that the treatment of the "4-4" pulp, while materially increasing its alpha cellulose content, tear, and color, does not materially affect its strength or pentosan content. In other words, the final pulp possesses the most valuable properties incident to both kraft and sulphite pulp, and may hence be beaten, sized and manufactured into high grade bond and ledger papers. The paper does not change color upon reasonable ageing in the air or upon exposure to light, and is substantially similar to ordinary "sulphite" paper in these respects.

I do not herein claim the subject matter 50 of application, Serial No. 716,154, filed May 27, 1924, or that of application, Serial No. 72,522, filed December 1, 1925 (both filed by Milton O. Schur and myself), which disclose the liberation of the usual sulphite pulp with the usual sulphite liquors, followed by a refining or purifying process to produce a high alpha cellulose fiber which comprises a pretreatment of the pulp with an oxidant, followed by digestion in an alkaline solution and bleaching. The sulphite liquors herein employed, in which the free SO<sub>2</sub> is not in excess of combined SO<sub>2</sub>, and in which the combined SO<sub>2</sub> amounts to about 3% to 4%, produce sulphite pulp 55 which when treated by the process of the

present invention yields a product having different characteristics than those products produced from pulp liberated with the usual sulphite liquors.

What I claim is:

1. A process which comprises digesting raw cellulosic material in an acid sulphite liquor in which the free SO<sub>2</sub> is not in excess of combined SO<sub>2</sub>, washing the resulting pulp substantially free from its digesting liquor, 70 treating said washed pulp with a solution containing chlorine, washing said chlorine-treated pulp, and digesting said washed and treated pulp at an elevated temperature in an alkaline solution. 75

2. In the manufacture of a pulp of high strength and whiteness, a process which comprises treating sulphite pulp, formed by previous digestion of raw cellulosic material in an acid sulphite liquor containing free and combined SO<sub>2</sub> in such proportion that such sulphite pulp is of extraordinary strength, with an oxidizing solution; washing said treated pulp; digesting said washed and treated pulp at an elevated temperature in 80 an alkaline solution; washing said digested pulp; and bleaching said washed pulp, said process substantially unaffected the strength of the sulphite pulp. 85

3. In the manufacture of a pulp of high strength and whiteness, a process which comprises treating sulphite pulp, formed by previous digestion of raw cellulosic material in an acid sulphite liquor containing free and combined SO<sub>2</sub> in such proportion that such sulphite pulp is of extraordinary strength, with an oxidizing solution; washing said treated pulp; digesting said washed and treated pulp at an elevated temperature in 90 an alkaline solution; washing said digested pulp, bleaching said washed pulp, and superbleaching said bleached pulp, said process substantially unaffected the strength of the sulphite pulp. 95

4. In the manufacture of a pulp of high strength and whiteness, a process which comprises treating sulphite pulp, formed by previous digestion of raw cellulosic material in an acid sulphite liquor containing free and combined SO<sub>2</sub> in such proportion that such sulphite pulp is of extraordinary strength, with a solution containing chlorine; washing said treated pulp, digesting said washed and treated pulp in a solution of sodium hydroxide; washing said digested pulp; and bleaching said washed pulp in hypochlorite bleach liquor, said process substantially unaffected the strength of the sulphite pulp. 110

5. In the manufacture of a pulp of high strength and whiteness, a process which comprises treating sulphite pulp, formed by previous digestion of raw cellulosic material in an acid sulphite liquor containing free and combined SO<sub>2</sub> in such proportion that such

sulphite pulp is of extraordinary strength, with a solution containing chlorine; washing said treated pulp, digesting said washed and treated pulp in a solution of sodium hydroxide; washing said digested pulp; bleaching said washed pulp in hypochlorite bleach liquor, and superbleaching said bleached pulp in a chlorine solution, said process substantially unafflicting the strength of the sulphite pulp.

6. In the manufacture of a pulp of high strength and whiteness, a process which comprises treating sulphite pulp, formed by previous digestion of raw cellulosic material in an acid sulphite solution in which the free  $\text{SO}_2$  and combined  $\text{SO}_2$  are in approximately equal proportions of 3% to 4% each with a solution containing about 2% to 4% chlorine based on the dry weight of fiber at about room temperature for about ten to thirty minutes; washing said treated pulp; digesting said washed and treated pulp in a caustic soda solution containing 6% to 8% caustic soda based on the dry weight of fiber at about 180° to 212° F. for about two to seven hours, washing said digested pulp; bleaching said pulp in a hypochlorite bleach solution containing 12% to 15% of 35% bleach ( $\text{CaOCl}_2$ ) based on the dry weight of fiber, at approximately room temperature for about five to ten hours, and superbleaching the bleached pulp in a chlorine solution containing about 0.3% chlorine based on the dry weight of fiber approximately at room temperature from two to six hours.

15 7. In the manufacture of a pulp of high strength and whiteness, a process which comprises digesting raw cellulosic material in an acid sulphite in which the free  $\text{SO}_2$  and combined  $\text{SO}_2$  are in approximately equal proportions of 3% to 4% each under conditions of high temperature and pressure, separating and washing the resulting pulp substantially free from its digesting liquor, treating said washed pulp with a solution containing chlorine, washing said chlorine-treated pulp, and digesting said washed and treated pulp at an elevated temperature in a solution of sodium hydroxide.

20 8. A process which comprises digesting raw cellulosic material in an acid sulphite in which the free  $\text{SO}_2$  and combined  $\text{SO}_2$  are in approximately equal proportions of 3% to 4% each under conditions of high temperature and pressure, separating and washing the resulting pulp substantially free from its digesting liquor, treating said washed pulp with a solution containing chlorine, washing said chlorine-treated pulp, and digesting said washed and treated pulp at an elevated temperature in a solution of sodium hydroxide.

25 9. In the manufacture of a pulp of high strength and whiteness, a process which comprises digesting raw cellulosic material in an acid sulphite in which the free  $\text{SO}_2$  and combined  $\text{SO}_2$  are in approximately equal proportions of 3% to 4% each with a solution containing about 2% to 4% chlorine based on the dry weight of fiber at about room temperature for about ten to thirty minutes; washing said treated pulp; digesting said washed and treated pulp in a caustic soda solution containing 6% to 8% caustic soda based on the dry weight of fiber at about 180° to 212° F. for about two to seven hours, washing said digested pulp; bleaching said pulp in a hypochlorite bleach solution containing 12% to 15% of 35% bleach ( $\text{CaOCl}_2$ ) based on the dry weight of fiber, at approximately room temperature for about five to ten hours.

30 10. In the manufacture of a pulp of high strength and whiteness, a process which comprises digesting raw cellulosic material in an acid sulphite in which the free  $\text{SO}_2$  and combined  $\text{SO}_2$  are in approximately equal proportions of 3% to 4% each with a solution containing about 2% to 4% chlorine based on the dry weight of fiber at about room temperature for about ten to thirty minutes; washing said treated pulp; digesting said washed and treated pulp in a caustic soda solution containing 6% to 8% caustic soda based on the dry weight of fiber at about 180° to 212° F. for about two to seven hours, washing said digested pulp; bleaching said pulp in a hypochlorite bleach solution containing 12% to 15% of 35% bleach ( $\text{CaOCl}_2$ ) based on the dry weight of fiber, at approximately room temperature for about five to ten hours.

35 11. In the manufacture of a pulp of high strength and whiteness, a process which comprises digesting raw cellulosic material in an acid sulphite in which the free  $\text{SO}_2$  and combined  $\text{SO}_2$  are in approximately equal proportions of 3% to 4% each with a solution containing about 2% to 4% chlorine based on the dry weight of fiber at about room temperature for about ten to thirty minutes; washing said treated pulp; digesting said washed and treated pulp in a caustic soda solution containing 6% to 8% caustic soda based on the dry weight of fiber at about 180° to 212° F. for about two to seven hours, washing said digested pulp; bleaching said pulp in a hypochlorite bleach solution containing 12% to 15% of 35% bleach ( $\text{CaOCl}_2$ ) based on the dry weight of fiber, at approximately room temperature for about five to ten hours.

40 12. In the manufacture of a pulp of high strength and whiteness, a process which comprises digesting raw cellulosic material in an acid sulphite in which the free  $\text{SO}_2$  and combined  $\text{SO}_2$  are in approximately equal proportions of 3% to 4% each with a solution containing about 2% to 4% chlorine based on the dry weight of fiber at about room temperature for about ten to thirty minutes; washing said treated pulp; digesting said washed and treated pulp in a caustic soda solution containing 6% to 8% caustic soda based on the dry weight of fiber at about 180° to 212° F. for about two to seven hours, washing said digested pulp; bleaching said pulp in a hypochlorite bleach solution containing 12% to 15% of 35% bleach ( $\text{CaOCl}_2$ ) based on the dry weight of fiber, at approximately room temperature for about five to ten hours.

In testimony whereof I have affixed my signature.

GEORGE A. RICHTER.